

## UNITED STATES PATENT OFFICE

1,980,377

PROCESS FOR REFINING AIRPLANE ENGINE  
OILArthur B. Brown and Arthur W. Neeley, Whiting,  
Ind., assignors to Standard Oil Company (Indiana), Chicago, Ill., a corporation of IndianaNo Drawing. Application September 12, 1930,  
Serial No. 481,594

10 Claims. (Cl. 196—44)

This invention relates to a process of making improved lubricating oils and especially high viscosity lubricating oils suitable for airplane engine lubrication. Because of the high temperatures at which airplane engines operate, it is necessary to provide a lubricating oil of high viscosity at ordinary temperatures and, in particular, one which will retain its viscosity at high temperatures. For this work, oils having a viscosity of between 90 and 150 seconds Saybolt at 210° F. are ordinarily employed. Furthermore, these oils must be abnormally stable to oxidation and sludging if they are to give satisfactory service under the severe conditions to which they are subjected.

The object of this invention is to provide a mineral lubricating oil which will retain its viscosity to a greater extent than any oil heretofore used for airplane lubrication, and further, to provide an airplane lubricating oil which will not be subject to sludging even after prolonged use at high temperatures. Another object of the invention is to provide an airplane lubricating oil having an extremely low content of non-combustible ash.

All lubricating oils are characterized by a reduction of viscosity with increase in temperature and some oils suffer a much greater loss of viscosity with increase in temperature than do others. In general, oils made from paraffin base crudes suffer the least change in viscosity with temperature, and are said to possess a low viscosity-temperature coefficient, whereas oils made from asphalt base crudes suffer the greatest change of viscosity with temperature, and are said to possess a high viscosity-temperature coefficient. Oils made from mixed base crudes occupy an intermediate position.

We have now discovered a method by which we can treat oils from mixed base crudes to substantially lower their viscosity-temperature coefficient. In fact, we have been able by using our method to reduce the viscosity-temperature coefficient of mixed base lubricating oils to that of paraffin base oils and even lower. Likewise, our process may be applied to paraffin base lubricating oils for the preparation of oils having a still lower viscosity-temperature coefficient.

In carrying out our invention we prefer to use as starting materials oils of high viscosity, as, for example, a 38% residuum from Mid-Continent crude. We may also employ a high viscosity distillate from Mid-Continent crude, preferably one having a viscosity between 150 and 300 seconds Saybolt at 210° F. Such a distillate may

be prepared by vacuum distillation, pipe-still distillation or other well-known method. When employing such a distillate in our process we obtain higher yields of finished oil with a somewhat lower chemical requirement than when residual oils are employed.

Having such an oil as a starting material, it is next subjected to a vigorous treatment with sulfuric acid. For this purpose we prefer to use fuming sulfuric acid of about 104.5%  $H_2SO_4$  grade. We have found, however, that lower acid concentrations may be employed with advantage for the first part of the treatment, if the treating is finished with fuming acid. Thus, we may treat the oil first with 93%  $H_2SO_4$  and finally with 104.5%  $H_2SO_4$ . With the weaker acid, we have found it advantageous to carry out the treatment at elevated temperature and a temperature of 180° F. has been found satisfactory. At this temperature, less acid may be used to obtain the same treating effect. With acid of this strength, however, there is a practical limit to the degree to which the viscosity-temperature coefficient can be reduced. Beyond that, it is necessary to use stronger acid and preferably fuming acid.

In our preferred procedure we subject the oil to a succession of acid treats as above, making a separation of the treated oil from sludge following each treat. A convenient quantity of acid to use in each treat is about one half pound per gallon of oil. Because of the high viscosity of the oil it is necessary to employ a suitable diluent, and for this purpose we have found it convenient to use a gas oil or kerosene stock prepared from straight distillation of Mid-Continent crude oil. This diluent is subsequently removed from the oil by distillation after the chemical process has been completed. The effect of the succession of acid treats on the viscosity-temperature coefficient of the oil is well illustrated by the following table which shows the ratio of Saybolt viscosity at 100° F. to viscosity at 210° F. for an oil of 120 seconds Saybolt viscosity at 210° F. made by treating 38% M. C. residuum with one pound of fuming acid per gallon in successive treats:

| Number of treats | Viscosity ratio |
|------------------|-----------------|
| None             | 18.0            |
| 2                | 15.7            |
| 3                | 14.1            |
| 4                | 12.6            |
| 5                | 11.0            |

105

110

The significance of these figures will be made apparent when compared with the viscosity ratio, 13.3, of a lubricating oil with a viscosity of 120 seconds Saybolt at 210° F. derived from paraffin base crude by the usual refining methods. We have found that oils most suitable for airplane engine lubrication should have a viscosity ratio of less than 15 and a Saybolt viscosity of 110-130 seconds at 210° F.

5 Although the oils prepared in the above manner are satisfactory from the standpoint of viscosity, it is difficult to refine them to acceptable ash content since they possess prohibitive quantities of oil soluble acids such as sulfonic acids 10 and other sulfuric acid derivatives, which, on neutralization, are converted into oil soluble soaps. These soaps are extremely difficult to remove from the viscous oil and, in fact, cannot be removed by any of the common methods such as 15 extraction with alkalis, alcohol, etc. After neutralization and alcoholic extraction, for example, these oils will contain sufficient soap to leave a non-combustible residue of from 0.5 to 1.3%. We have discovered that these refractory sulfonic acids and soaps can be successfully removed by 20 subjecting the oil to treatment with anhydrous aluminum chloride subsequent to the acid treatments above described. Although aluminum chloride has previously been used for treating 25 hydrocarbon oils, we believe we are the first to discover its unusual affinity for sulfonic acids. In addition to removing the sulfonic and other 30 objectionable organic acids, the aluminum chloride also assists in reducing the viscosity-temperature coefficient of the oil.

35

In using aluminum chloride, precautions must be taken to prevent access of water. If the oil is neutralized after the sulfuric acid treatment, it should be carefully dried for the subsequent aluminum chloride treats. In our preferred method, we do not neutralize the oil after sulfuric acid treating but after separating from the acid sludge we apply the aluminum chloride directly to the sour oil. The aluminum chloride is preferably applied in a succession of treats, and quantities of 0.3 pound per gallon of sour oil have been found suitable. One such treat is sufficient to reduce the ash from 0.8% to about 0.04%, and two such treats will reduce the ash to about 0.01%. The aluminum chloride treats may suitably be carried out at a temperature of 200 to 300° F. Somewhat lower temperatures may be employed but we avoid temperatures above 400° F. because of excessive cracking.

55 After the aluminum chloride treating, the oil is separated from the sludge, neutralized in the usual manner and dewaxed. The diluent may then be removed by distillation and the oil finally finished by treating it with a small quantity of fuller's earth. Or after separation from the aluminum chloride sludge, the oil may be treated with fuller's earth to obtain more complete sludge separation, thereafter neutralized, dewaxed and distilled to remove diluent. Either method yields an oil of high viscosity and negligible ash content which is remarkable for its excellent color, low viscosity-temperature coefficient and freedom from asphaltic constituents. Distillation may be carried out by use of vacuum, steam or other well known method to produce oils of the desired viscosity, either as bottom stocks or as overhead cuts. Wax may be removed by any of the usual methods either before or subsequent to removal of diluent.

75 The following example will illustrate the proc-

ess which is the subject of this invention as carried out on the large scale:

19,600 gallons of a distillate from Mid-Continent crude oil having a viscosity of 234 seconds Saybolt at 210° F. were diluted with 8,400 gallons of gas oil distillate. The mixture was then treated with one pound of 93% acid per gallon applied in two lots of one-half pound per gallon each, the sludge being separated after each treatment. The oil was then given two successive treats of one-half pound each of 104.5% fuming sulfuric acid per gallon of distillate. After the final acid sludge separation there remained 17,500 gallons of sour oil mixture. This oil was then treated with two successive lots of aluminum chloride of 0.4 pounds each per gallon of sour oil mixture at a temperature of 250° F. From four to eight hours were required for each treat, agitating the oil continuously during this time. The sludge was removed after each treatment and the oil was finally neutralized with caustic and distilled to the proper viscosity. The finished oil had a viscosity after dewaxing of 120 seconds at 210° F. and a viscosity ratio of 13.8. The color after treating with a small amount of fuller's earth was a pale fluorescent yellow and the ash content was 0.01%, whereas the ash content of the oil before the aluminum chloride treat was about 1%. This oil was tested in airplane engines and found to be superior to any oil previously employed, particularly from the standpoint of sustained viscosity and of freedom from sludge deposition in the crankcase and on the working parts of the engine.

After running for fifty hours with a jacket temperature of 300-350° F. and a crankcase temperature of 220-250° F., the viscosity of the oil which was originally 114 sec. Saybolt at 210° F. remained entirely unchanged showing no sludge formation nor polymerization by the high temperature. A standard paraffin base oil subjected to the same test increased in viscosity from 125 to 136 sec. at 210° F., and a standard mixed base airplane oil went from 126 to 186 sec. at 210° F. The latter oil developed an acidity three times that of our improved airplane oil and nearly twice the amount of insoluble sludge, the sludge formation being lower with our improved oil than with any other oil tested.

From the results of these and other tests, we believe we have discovered a method of making from mixed base crudes, lubricating oils with viscosity ratios substantially equivalent to those for paraffin base oils but with a degree of stability in airplane engine service surpassing that of any other oil known.

We have described our improved process in connection with a specific example thereof, but do not intend that it be limited thereby except as set forth in the following claims. 135

We claim:

1. The process of producing ash-free lubricating oils of low viscosity-temperature coefficient comprising subjecting a viscous lubricating oil admixed with a suitable diluent to a treatment with concentrated sulfuric acid sufficient to substantially reduce its viscosity-temperature coefficient and form undesirable sulfonic acids in the oil, separating the oil containing said sulfonic acids from the resulting acid sludge, then treating with anhydrous aluminum chloride in quantity sufficient to remove substantially all sulfonic acids present in the oil, separating the aluminum chloride sludge and neutralizing the oil.

2. The process of producing ash-free lubricat- 150

- ing oils of low viscosity-temperature coefficient from mixed base crudes comprising distilling the crude to produce a viscous lubricating oil, subjecting the viscous oil admixed with a suitable diluent to a treatment with concentrated sulfuric acid sufficient to substantially reduce its viscosity-temperature coefficient and form undesirable sulfonic acids in the oil, separating the oil containing said sulfonic acids from the resulting acid sludge, then treating the oil with anhydrous aluminum chloride in quantity sufficient to remove substantially all sulfonic acids present in the oil, separating the aluminum chloride sludge and finally finishing the oil by neutralizing, de-waxing, and distilling to the desired viscosity. 160° F. then treating with fuming sulfuric acid, separating the acid sludge after each successive treat and then treating the oil after the final acid treat with anhydrous aluminum chloride to remove sulfuric acid derivatives and further reduce the viscosity-temperature coefficient. 80
5. The method of removing oil-soluble organic acids from sulfuric acid-treated viscous mineral lubricating oils comprising treating the sour oil resulting from the acid treatments directly after removing the sulfuric acid sludge, with sufficient anhydrous aluminum chloride to remove the said organic acids. 85
6. The method of removing oil-soluble ash-forming sulfuric acid derivatives from viscous mineral lubricating oils having ash contents above 0.5% comprising treating the oil with sufficient anhydrous aluminum chloride to remove said sulfuric acid derivatives whereby the ash content of the oil is substantially reduced. 90
7. The method of removing oil-soluble ash-forming soaps from viscous mineral lubricating oils containing in excess of 0.5% ash comprising treating the oil with sufficient anhydrous aluminum chloride to remove said soaps, separating the resulting aluminum chloride sludge and neutralizing the remaining oil. 100
8. The method of removing from acid treated viscous mineral lubricating oils, oil soluble sulfuric acid compounds incapable of being removed by alcohol extraction, comprising treating the oil with sufficient anhydrous aluminum chloride to remove the said sulfonic acid compounds following the acid treatment and separating the resulting aluminum chloride sludge. 105
9. The process of reducing the viscosity-temperature coefficient of viscous mineral lubricating oils comprising successively treating with 93 to 100% sulfuric acid at a temperature above 110
4. The process according to claim 3 wherein the viscous lubricating oil employed is a crude oil residue. 115
5. The method of reducing the viscosity-temperature coefficient of viscous mineral lubricating oils comprising subjecting the oil to a succession of fuming sulfuric acid treats, separating the oil after each treat from the acid sludge, then treating the oil after the final acid treat with anhydrous aluminum chloride and neutralizing the resulting oil. 120
6. The process of reducing the viscosity-temperature coefficient of viscous mineral lubricating oils comprising successively treating with 93 to 100% sulfuric acid at a temperature above 125
- 40
- 45
- 50
- 55
- 60
- 65
- 70
- 75
- 130
- 135
- 140
- 145
- 150
- ARTHUR B. BROWN.  
ARTHUR W. NEELEY.